

## UNITED STATES PATENT OFFICE

2,012,866

## PYROTECHNIC COMPOSITION

Joseph B. Decker and Herbert C. Clouser,  
Elkton, Md.No Drawing. Application March 12, 1932,  
Serial No. 598,539

4 Claims. (Cl. 52—24)

This invention relates to a pyrotechnic composition designed to be employed in the manufacture of fireworks generally, in which the object is to obtain a spectacular flare or flash, with or without a detonative report, with a selective color range for the flash, and if desired, with the effusion of scintillating sparks or stars into the field of the flash.

The broad concept of the invention is the production of a combustible composition in which a rare earth metal or an element of periodic group IVa such for example as, zirconium, or an alloy of the same is burned in mixture with a suitable oxidizing agent.

It is old in the art to employ a compound of a rare earth metal or an element of periodic group IVa as an oxidant in mixture with some other combustible as a fuel, but since zirconium and others of the above indicated elements have a luminosity when burned far more brilliant than substances heretofore used for a similar purpose, it is obvious that the gist of the present invention lies in the fact of one of these substances or alloys of the same being used as the fuel and not as the oxidant.

Whether the combustion shall take the form of a flare or a flash depends upon the selection of the oxidant. Color may in a few instances be an attribute of the oxidant, but in general it is obtained by the addition to the mixture of a specific color producing ingredient. Detonation is produced by confining the mixture in a gas-tight shell or receptacle and whether it will explode by spontaneous fulmination or require ignition, as by a fuse, depends upon the fulminative sensitivity of the mixture, which is determined not only by the selection of the oxidant, but by the ratio of the detonative ingredient or its alloy to the oxidant.

Referring now to a detailed description of the invention, the detonating substance may be selected from the group exemplified by, zirconium, titanium, thorium, yttrium and selenium, and is employed in a comminuted state. It is characteristic of these elements and of their alloys that they burn with an exceptionally brilliant flame, that they enhance the combustive or fulminative sensitivity of the oxidizing agents with which they may be used in mixture, and that the sensitivity of the mixture depends not only

on the inherent nature of the oxidant, but also upon the quantity ratio of the rare earth metal or its alloy to the oxidant.

Taking zirconium for example, one part of this rare earth metal mixed with three parts of an oxidizing agent, such for instance, as barium nitrate, makes a flash mixture which explodes when ignited by a fuse, but which is not sufficiently sensitive to explode by impact.

By increasing the ratio of the zirconium to two parts to three, relative to the oxidant, a mixture is produced which readily explodes by impact. The sensitivity control afforded by varying the proportions of the rare earth metal or alloy relative to the oxidizing agent renders available a number of oxidizing agents of different co-efficients of sensitivity, such for example, as potassium nitrate, barium nitrate, oxalates, tri-nitro compounds, chlorates and perchlorates. The oxidizing agent is selected according to the use to which it is to be put. If the pyrotechnic device is of the type which is to be exploded, by impact, the oxidant is chosen with a view to giving the mixture a critical fulminative sensitivity, the detonating point of which can be very delicately determined by adjusting the quantity ratio of the oxidant to the detonative ingredient or alloy.

For example, by using a mixture of zirconium, two parts and barium nitrate, three parts, the exact proportions being adjusted to control the detonating point, a torpedo can be made so critical as to its fulminative sensitivity as to be altogether safe with respect to the shocks incident to its manufacture and transportation, and which will explode reliably under impact blows of a definite value above that of the incidental shocks referred to.

Where a particular color of the flash or flare is a desideratum, an oxidant is chosen which will produce a basic white color in the flame so that the imposed color will not be contaminated. For this purpose, the perchlorates are particularly suitable, for they not only burn the detonative ingredients with a white colorless flame which does not impair the purity of the imposed color, but they release a greater volume of gas, thus extending the field of the flash.

One of the important characteristics of the pyrotechnic composition of the present invention

is that it can have considerable proportions of other ingredients mixed with it without materially altering its co-efficient of combustive sensitivity. This makes it possible to add color-producing ingredients to the mixture without having to increase the ratio of the detonating elements or their alloys to the oxidizing agent.

An exemplary formula for a colored flash or flare would be:

- 10 -

Zirconium  
Perchlorates  
Strontium carbonate.

15 The last named ingredient gives a red color to the flash. The first two factors mixed in ratio of one to two give a mixture ignitable by a fuse, and in the ratio of two to three a mixture fulminating by impact.

35 Imp. 20. For producing stars or scintillating sparks in  
20 the field of flash, the detonative ingredient is  
ground coarser than when intended for in-  
stantaneous combustion. The larger granules do  
not consume immediately but are thrown out as  
highly incandescent burning particles or stars.  
25 Each of the elements has a spark of characteristic  
visual appearance. The zirconium spark for ex-  
ample, appears as an amoeba-shaped star, which  
shape is modified in alloys of zirconium. The  
characteristic sparks from burning iron appear  
30 as having thin radiating points. In a ferrous  
zirconium alloy, the shape of the spark is a com-  
promise between the zirconium and the iron  
sparks, the area of the amoeba-shaped star char-  
acteristic of zirconium being smaller, and the  
35 radiating points being thinner and more deeply  
indenting the central area.

A composition which includes in the mixture, several of the detonative ingredients exhibits an interesting variety of incandescent spark forms.

40 It is obvious from the above description that the new pyrotechnic composition is not confined

to any single field of application in the art of pyrotechnics, but that it is applicable to devices in which the composition is burned openly, without detonative effects, as in sparklers; in salutes which are ignited by a fuse, or in devices exploding upon impact, such as torpedoes.

What we claim is;

1. Pyrotechnic composition comprising a mixture of zirconium, and a perchlorate in proportion to detonate when confined, and a color imparting ingredient, the latter being present in such proportion as to give a decided color to the flash eventuating from the detonation of such mixture, the perchlorate functioning as an oxidizing agent.

2. Pyrotechnic composition with fulminating characteristic comprising a mixture of zirconium, a perchlorate, and a color producing ingredient, the perchlorate functioning as an oxidizing agent and the zirconium being comminuted to a degree of coarseness producing stars in the field of the flash eventuating from the detonation of said mixture. 15 20

3. Pyrotechnic composition capable of detonating comprising a mixture of an element selected from the following group, zirconium, titanium, thorium, yttrium, selenium, with an oxidizing agent, said element being comminuted to a state of sufficient coarseness to produce stars in the flash. 30

4. Pyrotechnic composition capable of detonating comprising a mixture of a fuel element selected from the following group: zirconium, titanium, thorium, yttrium, selenium with a perchlorate and a color producing agent used in sufficient proportion to produce a decided color in the flash, the fuel element being comminuted to such degree of coarseness as to produce stars in the flash. 35

JOSEPH B. DECKER. 40  
HERBERT C. CLAUSER.